

## UNITED STATES PATENT OFFICE

2,036,281

## PERMANENT MAGNET

Werner Köster, Dortmund, Germany, assignor, by  
mesne assignments, to Deutsche Edelstahlwerke  
Aktiengesellschaft, Crefeld, Germany

No Drawing. Application July 22, 1932, Serial  
No. 624,156. In Germany July 25, 1931

## 1 Claim. (Cl. 148—31)

This invention relates to a process for the treatment of ferromagnetic alloys.

The present invention constitutes a special application of the process for obtaining special magnetic properties in the case of ferromagnetic alloys, in which the solubility of a phase existing at room temperature increases as the temperature rises, said process forming the subject of my prior application No. 393,248 filed Sept. 17, 1929. The process according to the prior application consists in quenching the alloys from temperatures at which an increased formation of mixed crystals occurs and then leaving them alone or annealing them at a temperature below the quenching temperature. Thus, according to that process, iron alloys, for example, with an open gamma-field (such as iron-carbon alloys) are quenched from temperatures below the decomposition range of the austenite, whereas iron alloys with closed gamma-field (such as ferro-silicon, ferro-tungsten or the like) are quenched from temperatures between the commencement of the increased solubility and the melting point.

The subject of the present invention is the application of that process to special alloys and the employment of the alloys so treated for the production of permanent magnets.

Magnets have hitherto been manufactured from unalloyed or alloyed carbon steel, which was hardened in order to acquire its magnetic value. It has now been ascertained that, in applying the aforesaid process to the treatment of alloys intended for the production of permanent magnets, unexpectedly favourable properties are obtained by employing substantially carbon free ferromagnetic alloys hardened by precipitation hardening and containing 7 to 30% of at least one metal selected from the group tungsten and molybdenum together with 0.5 to 20% of cobalt, the balance of the alloy comprising substantially all iron.

These alloys receive their good properties, if they are first quenched from a temperature lying between about 900° C. and the melting point and then tempered at a temperature below the quenching temperature, preferably between about 500 and 800° C. Said treatment corresponds to the thermal treatment which is called precipitation hardening. At the quenching temperature the alloys consist of large, uniform mixed crystals which remains still after the quenching operation. During the tempering a second type of crystals is separating out, namely that type of crystals which are dissolved by annealing.

The different metallographic basis of the non-carbon or low-carbon steels of the present invention, as compared with existing magnetic steels introduces a series of new technical possibilities. After the first stage of heat treatment—quenching from high temperatures—these alloys are soft and easily worked, but are not yet usable magnetically, the magnetically favourable condition not being attained until the second stage of heat treatment, namely annealing at a moderate temperature. At the same time, the alloys become hard, but the hardness is such that they are also workable in this condition, though with more difficulty than in the quenched state.

The chromium, tungsten or cobalt magnetic steels hitherto customary are soft and workable only when in the annealed condition. On the other hand, they acquire martensitic hardness immediately after the quenching essential to their employment as magnets, and are therefore unworkable. In numerous cases, this constitutes a great drawback as regards shaping, especially in magnets of complicated form, or in the provision of fine bores, slots and cuts. Magnets made from the alloys of the present invention can, on the contrary, be roughly shaped, subjected to heat treatment and afterwards finished by machining. The work of finishing can be undertaken with particular ease after quenching. There is no risk of the magnets becoming distorted during the subsequent tempering, the changes of shape sustained in that operation being negligibly slight.

Another favourable factor in connection with the heat treatment of the alloys is that the alloys are practically free from carbon and therefore cannot exhibit, during the heat treatment, any phenomena of decarburization which may considerably injure the hitherto used carbon steels.

Further advantages of the alloys of the present invention are in respect of their magnetic properties. The nature of the heat treatment entirely precludes any change in structure during storage or slight heating, and these magnets are therefore not liable to age. By contrast, the martensitic structure of the existing magnetic steels is unstable, and its coercitvity is considerably diminished even by tempering at moderate temperatures. The alloys of the present invention, on the other hand, can be heated to redness without impairing their magnetic value (measured at room temperature). A further consequence is that the same value is maintained at each temperature when heating and cooling,

**2**

whereas, with the old magnet steels, lower values are obtained in cooling than in heating.

The following examples will serve to illustrate the invention:

*Example 1*

5 An alloy of 9.8% of cobalt, 18.2% of tungsten, 1.4% of vanadium and 0.04% of carbon gave, after quenching from 1275° C., a coercive force of 4 Gauss, a remanence of 4200 Gauss and a Brinell hardness value 320. After tempering for 30 minutes at 750° C., the coercive force became 108 Gauss, the remanence 11750 Gauss and the hardness 550.

*Example 2*

15 An alloy with 5.2% of cobalt, 15.6% of molybdenum, 0.6% of vanadium and 0.04% of carbon

gave, after quenching from 1100° C. and tempering for 30 minutes at 700° C., the coercive force 116 Gauss and remanence 11500 Gauss.

The balance of the alloy consists in each example principally of iron.

5

## I claim:—

Permanent magnets composed of a substantially carbon free ferro-magnetic alloy hardened by precipitation hardening and containing 7 to 30% of at least one metal selected from the group 10 tungsten and molybdenum together with 0.5 to 20% of cobalt, the balance of the alloy comprising substantially all iron, said alloy having such improved magnetic qualities which are caused by precipitation hardening of such alloy. 15

WERNER KÖSTER.